

## [54] FLAME SPRAY POWDER

- [75] Inventors: **Paul A. Kammer**, Cold Spring Harbor; **George Yurasko, Jr.**, Glen Cove; **Karel Zmrzlik**, New York, all of N.Y.
- [73] Assignee: **Eutectic Corporation**, Flushing, N.Y.
- [21] Appl. No.: **251,331**
- [22] Filed: **Apr. 6, 1981**
- [51] Int. Cl.<sup>3</sup> ..... **B05D 1/10**
- [52] U.S. Cl. ..... **427/423; 75/251**
- [58] Field of Search ..... **75/251; 427/423**

## [56] References Cited

## U.S. PATENT DOCUMENTS

- 3,436,248 4/1969 **Dittrich et al.** ..... 427/423
- 4,031,278 6/1977 **Patel** ..... 427/423
- 4,166,736 9/1979 **Bewley** ..... 75/251 X
- 4,168,967 9/1979 **Sridhar et al.** ..... 76/362 X

Primary Examiner—Shrive P. Beck

*Attorney, Agent, or Firm*—Hopgood, Calimafde, Kalil, Blaustein & Judlowe

## [57]

## ABSTRACT

A free-flowing self-bondable flame spray powder derived from an atomized alloy powder is provided in which the particles are characterized by aspherical shapes and have an average particle size within the range of about plus 400 mesh to minus 100 mesh. The aspherically shaped powder is further characterized by a specific surface of about 180 cm<sup>2</sup>/gr and higher and has a composition consisting essentially of a solvent metal of melting point in excess of about 1100° C. whose negative free energy of oxidation ranges up to about 80,000 calories per gram atom of oxygen referred to 25° C. The solvent metal contains at least one highly oxidizable solute metal in an amount of at least about 3% by weight, the oxidizable metal having a negative free energy of oxidation of at least about 100,000 calories per gram atom of oxygen referred to 25° C.

12 Claims, 2 Drawing Figures



60X



80X

**FIG. 1**



80X

**FIG. 2**

## FLAME SPRAY POWDER

This invention relates to a self-bonding flame spray alloy powder, otherwise referred to herein as a one-step flame spray powder.

## STATE OF THE ART

It is known to coat metal substrates with a flame spray material to protect said metal substrates, such as a ferrous metal substrate, including steel and the like, and impart thereto improved properties, such as resistance to corrosion, and/or oxidation, and/or wear, and the like. The material sprayed, e.g., metals, may be in the form of a wire or a powder, powder spraying being a 15 preferred method.

In order to provide a substrate with an adherent coating, it is the practice to clean the substrate and prepare the surface by shot blasting it with steel grit or by threading the surface on a lathe, if the shape is cylindrical, before depositing the metal coating thereon.

In U.S. Pat. No. 3,322,515, a method is disclosed for providing an adherent coating onto a metal substrate by first cleaning the substrate and flame spraying a metal bond coat thereon using a flame spray powder in which 20 elemental nickel and aluminum are combined together to form a composite particle, for example, a clad particle. This type of powder which is referred to in the trade as bond coat powder provides a basis layer by means of which a sprayed overlayer of other metals and 25 alloys of substantial thickness is adherently bonded to the metal substrate. With this technique, fairly thick overlayers can be produced.

According to the patent, the nickel and aluminum in the composite particles are supposed to react exothermically in the flame to form an intermetallic compound (nickel aluminide) which gives off heat which is intended to aid in the bonding of the nickel-aluminum material to the metal substrate, the intermetallic compound forming a part of the deposited coating.

It is known in the patent literature to employ aluminum powder simply mixed with the particulate coating material to enhance the flame spraying thereof by using the heat of oxidation of aluminum which is substantially greater than the amount of heat released in the formation of the nickel aluminide intermetallic compound. A patent utilizing the foregoing concept is the Bradstreet U.S. Pat. No. 2,904,449 which discloses the use of a flame catalyst, e.g., aluminum, capable of catalyzing the oxidation reaction being carried out in the flame to thereby raise the flame temperature. Another patent along substantially the same line is Haglund U.S. Pat. No. 2,943,951.

In U.S. Pat. No. 4,230,750, a method is disclosed for producing an adherent coating using a flame spray powder mixture comprising: (1) agglomerates of a metallo-thermic heat-generating composition comprised essentially of fine particles of a reducible metal oxide formed from a metal characterized by a free energy of oxidation ranging up to about 60,000 calories per gram atom of oxidation referred to 25° C. intimately combined together by means of a thermally fugitive binder with fine particles of a strong reducing agent consisting essentially of a metal characterized by a free energy of oxidation referred to 25° C. of at least about 90,000 calories 65 per gram atom of oxygen, (2) said agglomerates being uniformly mixed with at least one coating material selected from the group consisting of metals, alloys, and

oxides, carbides, silicides, nitrides, and borides of the refractory metals of the 4th, 5th, and 6th Groups of the Periodic Table.

According to the patent, by employing a metallo-thermic heat generating composition (i.e., a thermit mixture) in agglomerated form and simply mixing it with a coating material, e.g., nickel, among other coating materials, markedly improved bonding results are obtained as compared to using the agglomerated metallo-thermic composition alone followed by a sprayed overlayer.

By employing the metallo-thermic agglomerate, different flame characteristics are obtained which are conducive to the production of strongly adherent coatings.

In U.S. Pat. No. 4,039,318, a metaliferous flame spray material is disclosed, formed of a plurality of ingredients physically combined together in the form of an agglomerate, the plurality of ingredients in the agglomerate comprising by weight of about 3% to 15% aluminum, about 2 to 15% refractory metal silicide and the balance of the agglomerate essentially a metal selected from the group consisting of nickel-base, cobalt-base, iron-base, and copper-base metals. A preferred combination is at least one refractory metal disilicide, e.g., TiSi<sub>2</sub>, agglomerated with aluminum and nickel powder. The foregoing combination of ingredients provides metal coatings, e.g., one-step coatings, having improved machinability.

A disadvantage of using composite powders comprising elemental nickel and aluminum particles bonded together with a fugitive binder is that the coating obtained is not a completely alloyed coating as evidenced by the presence of free aluminum in the coating. Such coatings are not desirable for providing corrosion resistant properties.

It is known to produce coatings from alloy powders, particularly alloy powders in which one of the alloying constituents is a solute metal of a highly oxidizable metal, such as aluminum. A typical alloy is an atomized powder containing nickel as a solvent metal alloyed with 5% aluminum. Gas atomized powders are employed in that such powders, which are generally spherical in shape, are free-flowing which is desirable for flame spraying. In order to assure bonding, relatively high flame spray temperatures are required. Thus, 30 plasma torches are preferred in order to consistently produce coatings having the desired bond strength. The residence time during flight through the plasma or gas flame is very short and requires rapid heat absorption by the flame spray powder in order to reach the desired 35 temperature. Thus, in the case of flame spraying with an oxyacetylene torch, it was not always possible to obtain consistently the desired bond strength, although such coatings were very desirable in that they were truly alloy coatings with the aluminum substantially dissolved in or pre-reacted with the solvent nickel.

We have now found that we can overcome the foregoing bonding problem with alloy powders of the aforementioned or similar compositions by employing alloy powders having a particle configuration characterized by a high specific surface as compared to the relatively lower specific surface of gas-atomized alloy powders having a substantially spherical shape, when such powders are compared over substantially the same particle size distribution.

## OBJECTS OF THE INVENTION

It is an object of the invention to provide an alloy flame spray powder capable of producing adherent

coatings on metal substrates characterized by improved bond strength.

Another object is to provide a method for flame spraying an adherent one-step coating using an alloy flame spray powder.

These and other objects will more clearly appear when taken in conjunction with the following disclosure, the appended claims, and the accompanying drawings, wherein:

FIG. 1 is a representation of a photomicrograph taken at 80 times magnification of a gas-atomized flame spray alloy powder showing very smooth particles of substantially spherical shape; and

FIG. 2 is a representation of a photomicrograph taken at 80 times magnification of a flame spray alloy powder atomized to provide particles having a randomly irregular aspherical configuration characterized by high specific surface.

#### STATEMENT OF THE INVENTION

In its broad aspects, the invention is directed to a flame spray powder derived from an atomized alloy in which the particles are characterized by aspherical shapes and have an average particle size falling in the range of about 400 mesh to minus 100 mesh (U.S. Standard), e.g., about 35 to 150 microns, the aspherically shaped powder being further characterized by a specific surface of about 180  $\text{cm}^2/\text{gr}$  and generally about 250  $\text{cm}^2/\text{gr}$  and higher. By specific surface is meant the total average surface area of particles per gram of the particles.

The alloy powder is characterized by a composition consisting essentially of a solvent metal of melting point in excess of about 1100° C. whose negative free energy of oxidation ranges up to about 80,000 calories per gram atom of oxygen referred to 25° C. and contains at least one highly oxidizable solute metal as an alloying constituent in an amount of at least about 3% by weight, said oxidizable metal having a negative free energy of oxidation of at least about 100,000 calories per gram atom of oxygen referred to 25° C.

Examples of solvent metals are the iron-group metals, nickel, iron, and cobalt and the iron-group base alloys, nickel-base, iron-base, and cobalt-base alloys and mixtures thereof. Examples of highly oxidizable solute metals are aluminum, titanium, zirconium, and the like, the highly oxidizable metals being characterized by a free energy of oxidation of at least about 100,000 calories per gram atom of oxygen as stated hereinabove.

The term "solvent metal" is meant to cover iron-group metals per se and iron-group metal base alloys. It is understood that the solvent metals may contain one or more alloying ingredients, such as chromium, molybdenum, tungsten, etc., so long as the iron-group metals are predominant and the alloys are less oxidizing than the highly oxidizable solute metal.

The presence of the highly oxidizable solute metal is important together with the configuration of the atomized powder in providing the property of self-bonding when the powder is flame sprayed.

It has been found that by employing randomly irregular aspherical powders having a specific surface of about 180  $\text{cm}^2/\text{gr}$  and higher, and preferably at least about 250  $\text{cm}^2/\text{gr}$ , the powder is capable of high heat absorption during the short residence time in the flame, such that the particles striking the substrate are at the desirable temperature conducive to self-bonding. The

presence of the highly oxidizable solute metal also aids in providing self-bonding characteristics.

It is important that the average particle size be controlled over the range of about 400 mesh to minus 100 mesh (about 35 to 150 microns) and preferably from about 325 mesh to 140 mesh (about 45 to 105 microns). The particles may be spherical gas-atomized powder which has been later flattened by ball milling so as to increase the specific surface; or the aspherical particles may be atomized powder formed by water, steam or gas atomization, such that the ultimate powder has a randomly irregular aspherical shape of high specific surface.

The term "average size" means the average of the minimum and maximum size of the aspherical particles. For example, some of the particles may be less than about 400 mesh (less than about 35 microns) so long as the average size is over about 400 mesh. Similarly, some of the particles may be in excess of 100 mesh (in excess of about 150 microns) in size so long as the overall average size is 100 mesh or less.

Besides being aspherical, the powder should be free-flowing so as to assure gravity feed to a torch. Thus, the apparent density of the powder and its size should not be so low as to lose its free-flowing characteristics.

Moreover, the average particle size should not fall substantially below 400 mesh, otherwise the alloy powder tends to oxidize and burn up in an oxyacetylene flame.

#### DETAILS OF THE INVENTION

The importance of powder configuration in carrying out the purposes and aims of the invention has been confirmed by tests in which the bonding characteristics of gas-atomized spherical powder were compared to randomly irregular aspherical particles.

Substantially spherical particles in the range of about 400 mesh to 100 mesh do not provide adequate specific surface to assure relatively high bonding strength.

However, when the atomized particles are flattened, as by ball milling, the specific surface per gram of powder can be substantially increased. Substantially the same effect can be achieved by specially atomizing the alloy by high pressure water, steam or gas in a manner conducive to produce randomly irregular aspherical particles characterized by a high specific surface.

As illustrative of substantially spherical gas-atomized particles, reference is made to FIG. 1 which is a representation of a photomicrograph taken at about 80 times magnification.

Assuming a particle size distribution of spherical particles falling in the range of about 400 mesh to 100 mesh (e.g., about 35 to 150 microns), the specific surface in  $\text{cm}^2/\text{gr}$  is determined for an alloy of 95NI-5Al having a density of about 8.283 (d) as follows, the diameter (D) of the spherical particles being given in microns:

$$S.S. = \frac{\pi D^2}{1/6\pi D^3 \times d} = \frac{6}{Dd}$$

Converting to centimeters, the formula is as follows:

$$S.S. = \frac{6 \times 10^4}{D \times 8.283} = \frac{7244}{D} \text{ cm}^2/\text{gr}$$

Assuming that the spherical particles in the range of 400 to 100 mesh (U.S. Standard) are flattened to a thickness of about 10 microns and have substantially a circular shape, the change in specific surface from the spherical configuration to the flattened configuration will be apparent from the following table:

| MESH | DIAM.<br>ATOMIZED<br>SPHERICAL<br>POWDER | SURFACE<br>AREA<br>SPECIFIC | PARTICLES<br>FLATTENED TO 10<br>MICRONS THICK |                     |
|------|------------------------------------------|-----------------------------|-----------------------------------------------|---------------------|
|      |                                          |                             | DIAM. OF<br>DISC (μ)                          | SPECIFIC<br>SURFACE |
|      |                                          |                             |                                               | MICRONS             |
| 100  | 149                                      | 48.6                        | 470                                           | 251.7               |
| 120  | 125                                      | 57.9                        | 362                                           | 254.7               |
| 140  | 105                                      | 69.0                        | 272                                           | 259.2               |
| 170  | 88                                       | 82.3                        | 255                                           | 260.3               |
| 200  | 74                                       | 97.9                        | 160.2                                         | 271.5               |
| 230  | 62                                       | 116.8                       | 126.5                                         | 279.6               |
| 270  | 53                                       | 136.7                       | 81.4                                          | 300.7               |
| 325  | 44                                       | 164.6                       | 75.5                                          | 305.4               |
| 400  | 37                                       | 195.8                       | 58.3                                          | 324.2               |
| —    | 30                                       | 241.5                       | 42.4                                          | 355.3               |

The particles after flattening are deemed to be disc-shaped, although it will be appreciated that some of the particles may have a slightly elliptical shape.

As has been stated herein, the average particle size of the flame spray powder should range from 400 to 100 mesh (about 35 to 150 microns).

According to the table, the usable powder of high specific surface (e.g., about 180 cm<sup>2</sup>/gr or at least about 250 cm<sup>2</sup>/gr) are those powders whose particle size, following flattening, ranges from about 42 to 126 microns (or about 325 to 120 mesh). The desired particles of flattened configuration are obtained by sieving to provide sizes in the range of approximately 325 to 120 mesh (e.g., over 42 to about 125 microns) these powders being derived from gas-atomized alloy powders.

Particles of high specific surface can be provided by employing atomizing techniques using water, gas or steam as the atomizing agent under conditions which favor the formation of irregular particles. Thus, in the case of water atomization, the conditions are easily determined by setting the pressure and flow rate of the fluid according to nozzle design so as to produce turbulent forces which override the normal sphere-forming surface tension forces acting on the molten particle. An advantage of water atomization is its high quenching rate capability which causes the particles to freeze rapidly into irregular aspherical shapes. In the case of gas atomization, cool gases may be employed.

As illustrative of an irregularly shaped atomized alloy powder, reference is made to FIG. 2 which shows particles of relatively high specific surface having randomly irregular aspherical shapes. Such atomized powders are characterized as having free-flowing properties for use in flame spray torches, such as oxyacetylene torches of the type disclosed in U.S. Pat. Nos. 3,986,668 and 3,620,454, among others, depending on the feed rate employed and energy capacity of the torch.

By using aspherical powder of the composition disclosed herein in accordance with the invention, relatively high bonding strengths in excess of about 2000 psi, e.g., of about 2500 psi and above, are obtainable as measured in accordance with ASTM C633-69 Procedure.

According to the ASTM Procedure, the determination is made by using a set of two cylindrical blocks one inch in diameter and one inch long. An end face of each

block of the set is ground smooth and one face first coated with the aforementioned bond coat compositions by flame spraying to a thickness of about 0.008 to 0.012 inch. A high strength overcoat is applied to the first coat, the high strength overcoat being, for example, a nickel-base alloy known by the trademark Inconel (7% Fe-15% Cr—balance Ni) of a type 431 stainless steel (16% Cr and the balance iron). The thickness of the high strength overcoat is about 0.015 to 0.020 inch; and after depositing it, the overall coating which has a thickness ranging up to about 0.025 inch is then finished ground to about 0.015 inch. A layer of epoxy resin is applied to the overcoat layer, the epoxy layer having a bond strength of over 10,000 psi.

The other block of the set is similarly end ground to a smoothness corresponding to 20 to 30 rms and layer of high strength epoxy resin applied to it. The two blocks of the set are assembled together by clamping one with the metal coating and the epoxy layer to the other, with the epoxy faces of the blocks in abutting contact, and the clamped blocks then subjected to heating in an oven to 300° F. (150° C.) for one hour, whereby the epoxy faces strongly adhere one to the other to provide a strongly bonded joint.

The joined blocks are then pulled apart using anchoring bolts coaxially mounted on opposite ends of the joined blocks using a tensile testing machine for recording the breaking force. The bonding strength is then determined by dividing the force obtained at failure by the area of the one inch circular face of the blocks.

As illustrative of the invention, the following examples are given:

#### EXAMPLE 1

A test was conducted based on an alloy of 95% Ni-5% Al in which a coating produced from a gas-atomized alloy powder of substantially spherical shape was compared to the coating of the same alloy powder flattened out by ball milling and to a coating of the same composition produced by a water atomization under conditions to provide particles having a randomly irregular spherical shape of high specific surface, the three alloy powders having an average size ranging from about 325 mesh to 140 mesh. All of the powders had the desired free-flowing characteristics and were flame sprayed using an oxyacetylene torch referred to by the trademark Rotoloy of the type disclosed in U.S. Pat. No. 3,986,668.

The powders were fed at a rate of about 5 to 6 lbs./hour and were deposited on a substrate of 1020 steel. The bond strength was measured in accordance with ASTM C633-69 as described hereinabove. The surface area of the powder was determined using the BET method. The correlation of the powders relative to the specific surface and the bonding strength is as follows:

TABLE 1

|     | Type of Powder                            | Specific Surface         | Bond Strength             |
|-----|-------------------------------------------|--------------------------|---------------------------|
| (1) | Gas-atomized spherical particles          | 174 cm <sup>2</sup> /gr* | 1250 lbs./in <sup>2</sup> |
| (2) | Same as (1) but ball milled to flat shape | 341 cm <sup>2</sup> /gr  | 2700 lbs./in <sup>2</sup> |
| (3) | Specially water-                          | 961 cm <sup>2</sup> /gr  | 2700 lbs./in <sup>2</sup> |

TABLE 1-continued

| Type of Powder  | Specific Surface | Bond Strength |
|-----------------|------------------|---------------|
| atomized powder |                  |               |

\*The specific surface value of powder (1) indicates that the atomized particles are not perfect spheres; however, the value is almost one-half the value of powder (2) produced by ball milling powder (1).

As is clearly apparent from the table, the powders with the relatively high specific surface in excess of 180 cm<sup>2</sup>/gr provide markedly improved bonding strength.

However, particle shape is not the only important consideration. It is also important that the alloy contain a highly oxidizable metal, such as aluminum, as stated hereinabove. This is illustrated by tests conducted under the same conditions using particles of nickel per se of different specific surface, (1) a chemically produced powder of high specific surface having an average size ranging from about 325 mesh to 140 mesh, and (2) an atomized nickel powder of irregular shape.

The results obtained are as follows:

TABLE 2

| Type Nickel Powder                     | Specific Surface         | Bond Strength (psi) |
|----------------------------------------|--------------------------|---------------------|
| (1) Chemically produced powder         | 1940 cm <sup>2</sup> /gr | <200                |
| (2) Irregularly shaped atomized powder | 670 cm <sup>2</sup> /gr  | <200                |

As will be noted, each of powders (1) and (2) have a specific surface substantially in excess of 180 cm<sup>2</sup>/gr, e.g., in excess of 600 cm<sup>2</sup>/gr, yet the bonding strengths of all two powders were below 200 lbs./in<sup>2</sup>, thus signifying the importance of the presence of aluminum in the alloy powder of Table 1.

Free-flowing characteristics of the flame spray powder are important. The desirable free-flowing characteristics are those defined by the flow rate of a predetermined amount of powder through a funnel, such as the well-known Hall Flow Rate.

The Hall Flow Rate device comprises an inverted cone or funnel having an orifice at the bottom of the funnel or cone of one-tenth inch diameter and a throat one-eighth inch long. Such a funnel is illustrated on page 50 of the Handbook of Powder Metallurgy by Henry H. Hausner (1973, Chemical Publishing Co., Inc., New York, NY). The flow rate is the number of seconds it takes 50 grams of powder to pass through the opening of the funnel. A typical flow rate of a randomly irregular aspherical powder as illustrated in FIG. 2 is 30 to 33 seconds for 50 grams of powder having the following particle distribution:

| MESH | WT. %     |
|------|-----------|
| +100 | 0         |
| +140 | 1.0 max.  |
| +170 | 10.0 max. |
| +325 | bal.      |
| -325 | 20.0 max. |

#### EXAMPLE 2

Another alloy composition tested in accordance with the invention is one containing about 15% Al and the balance essentially nickel. The alloy was water-atomized to produce a high specific area.

The results obtained are given in Table 3 below.

TABLE 3

| Alloy Powder | Specific Surface         | Bond Strength (psi) |
|--------------|--------------------------|---------------------|
| Ni - 15% Al  | 2430 cm <sup>2</sup> /gr | 4200                |

A test conducted with an alloy of Ni-3% Ti (density of 8.59 grs/cc) indicated that the presence of titanium appears to have a stronger beneficial effect on bonding than aluminum, even at a specific surface of about 160 cm<sup>2</sup>/gr, a bond strength of 5100 psi being obtained. However, it is preferred for consistent results that the specific surface be about 180 cm<sup>2</sup>/gr and above.

An advantage of producing a one-step alloy coating or a bond coat in accordance with the invention is that the deposited alloy coating is generally homogeneous and does not contain free aluminum as does occur when spraying composite powders comprising agglomerates of elemental nickel and aluminum.

Examples of various Ni-base, Co-base and Fe-base alloy compositions that can be sprayed so long as the powder particles are configurated to provide high specific surface are given as follows:

| % Ni | % Co | % Fe | % Al | % Ti |
|------|------|------|------|------|
| 90   | —    | —    | 5    | 5    |
| 97   | —    | —    | —    | 3    |
| 92   | —    | —    | 5    | 3    |
| —    | 85   | —    | 15   | —    |
| —    | 90   | —    | 5    | 5    |
| —    | —    | 95   | 5    | —    |
| —    | —    | 94   | 3    | 3    |

A preferred alloy is one containing about 4% to 20% aluminum or about 4% to 10% aluminum and the balance nickel.

Although the present invention has been described in conjunction with preferred embodiments, it is to be understood that modifications and variations thereto may be resorted to without departing from the spirit and scope of the invention as those skilled in the art will readily understand. Such modifications and variations are considered to be within the purview and scope of the invention and the appended claims.

What is claimed is:

1. A free-flowing self-bondable flame spray powder derived from an atomized alloy, said powder having particles characterized by aspherical shapes and having an average particle size within the range of about plus 400 mesh to minus 100 mesh, said aspherically shaped powder being further characterized by a specific surface of about 180 cm<sup>2</sup>/gr and higher, said flame spray powder having a composition consisting essentially of a solvent metal of melting point in excess of about 1100° C. whose negative free energy of oxidation ranges up to about 80,000 calories per gram atom of oxygen referred to 25° C. and being pre-alloyed with at least one highly oxidizable solute metal in an amount of at least about 3% by weight, said oxidizable metal having a negative free energy of oxidation of at least about 100,000 calories per gram atom of oxygen referred to 25° C.

2. The free-flowing self-bondable flame spray powder of claim 1, wherein the average particle size of said aspherical powder ranges from about 325 mesh to 140 mesh, wherein the amount of said oxidizable metal ranges from about 4% to 20% by weight of said alloy

powder and wherein the specific surface of the powder is about 250 cm<sup>2</sup>/gr and higher.

3. The free-flowing powder of claim 2, wherein said solvent metal is selected from the metals consisting of iron-group Ni, Fe, Co, and iron-group base alloys Ni-base, Fe-base, Co-base alloys and mixtures thereof.

4. A free-flowing one-step self-bondable atomized flame spray powder having particles characterized by randomly irregular aspherical shapes and having an average particle size ranging from about 325 mesh to 140 mesh,

said randomly irregular aspherically shaped powder being further characterized by a specific surface of about 250 cm<sup>2</sup>/gr and higher,

said atomized flame spray powder being formed of a solvent alloy selected from the iron-group base alloys consisting of Ni-base, Fe-base, Co-base alloys and mixtures thereof of melting point in excess of 1100° C. whose negative free energy of oxidation ranges up to about 80,000 calories per gram atom of oxygen referred to 25° C. and being pre-alloyed with about 4% to 20% by weight of a highly oxidizable solute metal whose free energy of oxidation is at least about 100,000 calories per gram atom of oxygen referred to 25° C.

5. The free-flowing flame spray powder of claim 4, wherein the solvent alloy is essentially nickel and said solute metal is aluminum ranging in amount from about 4% to 20% by weight.

6. The free-flowing flame spray powder of claim 4, wherein the solvent alloy is essentially nickel containing about 4% to 10% aluminum.

7. A method of producing an adherent metal coating on a metal substrate, said method comprising flame spraying a free-flowing powder derived from an atomized alloy and having particles characterized by aspherical shapes and an average particle size within the range of about plus 400 mesh to minus 100 mesh,

said aspherically shaped powder being further characterized by a specific surface of about 180 cm<sup>2</sup>/gr and higher,

said flame spray powder having a composition consisting essentially of a solvent metal of melting point in excess of about 1100° C. whose negative free energy of oxidation ranges up to about 80,000 calories per gram atom of oxygen referred to 25° C. and being

pre-alloyed with at least one highly oxidizable solute metal in an amount of at least about 3% by weight, said oxidizable metal having a free energy of oxidation of at least about 100,000 calories per gram atom of oxygen referred to 25° C., and continuing said flame spraying to form an adherent alloy coating on said metal substrate.

8. The flame spray method of claim 7, wherein the average particle size of aspherical powder being sprayed ranges from about 325 mesh to 140 mesh and wherein the amount of said highly oxidizable metal ranges from about 4% to 20% by weight of said alloy powder.

9. The flame spray method of claim 8, wherein the alloy sprayed is selected from the group consisting of the iron-group metals Ni, Co, Fe and Ni-base, Co-base and Fe-base alloys and mixtures thereof.

10. A method of producing an adherent metal coating on a metal substrate, said method comprising flame spraying a free-flowing atomized powder having particles characterized by randomly irregular aspherical shapes and having an average particle size ranging from about 325 mesh to 140 mesh,

said randomly irregular aspherically shaped powder being further characterized by a specific surface of about 250 cm<sup>2</sup>/gr and higher,

said atomized flame spray powder being formed of a solvent alloy selected from the group consisting of the iron-group alloys Ni-base, Co-base, Fe-base alloys and mixtures thereof of melting point in excess of 1100° C. whose negative free energy of oxidation ranges up to about 80,000 calories per gram atom of oxygen referred to 25° C. and being pre-alloyed with about 4% to 20% by weight of a highly oxidizable solute metal whose free energy of oxidation is at least about 100,000 calories per gram atom of oxygen referred to 25° C.,

and continuing said flame spraying to form an adherent metal coating on said metal substrate.

11. The flame spray method of claim 10, wherein the alloy being sprayed employs nickel as the solvent metal and aluminum as the solute metal.

12. The flame spray method of claim 11, wherein the alloy being sprayed contains about 4% to 10% aluminum.

\* \* \* \* \*